

## [54] RADIOISOTOPE FUEL MATERIAL AND METHOD

[75] Inventor: Vahe Keshishian, Sherman Oaks, Calif.

[73] Assignee: Rockwell International Corporation, El Segundo, Calif.

[\*] Notice: The portion of the term of this patent subsequent to June 2, 1987, has been disclaimed.

[22] Filed: Jan. 13, 1971

[21] Appl. No.: 106,071

## Related U.S. Application Data

[60] Continuation of Ser. No. 815,131, April 10, 1969, which is a continuation-in-part of Ser. No. 687,945, Oct. 25, 1967, which is a division of Ser. No. 464,702, June 17, 1965, Pat. No. 3,515,875.

[52] U.S. Cl. .... 252/301.1 R, 423/249, 423/250, 423/251, 423/252, 423/253, 136/202

[51] Int. Cl. .... C01g 56/00

[58] Field of Search .... 252/301.1 R; 23/343-347, 354-355; 136/202

## [56] References Cited

## UNITED STATES PATENTS

3,420,640 1/1969 Porter ..... 23/344

## OTHER PUBLICATIONS

Argo, et al.; Neutron Emission by Polonium Oxide Layers, Nuc. Sci. Abs., Vol. 10, No. 11, Abs. No. 3648, 1956, p. 464.

Terent'Ev, Polonium Oxides, Nuc. Sci. Abs., Vol. 10, No. 17, 1956, p. 791.

Richter, Ceramic Tubes Developed For External Heat Sources, Nuc. Sci. Abs., Vol. 15, No. 18A, Abs. No. 23676, 1961 p. 3053.

"Snap Programs", Nuc. Sci. Abs., Vol. 15, No. 10, 1961, Abs. No. 12652, p. 1620.

Madorsky, et al., Concentration of Isotopes of C1 by the Counter-Current Electromigration Method, J. of Research, N.B.S., Vol. 38, 1947, p. 185.

Kistemaker et al., Proc. of the Internat. Symposium on Isotope Separation, 1958, pp. 158, 336, 337.

Calvin, et al., Isotopic Carbon, 1949, Wiley &amp; Sons, p. 4.

"Stable Isotopes", USAEC Publication, 1948.

Sheft, et al., Equilibrium in the Vapor-Phase Hydrolysis of Plutonium Trichloride, The Transuranium Elements, McGraw Hill, 1949, pp. 841-847.

Keshishian et al., Use of O<sup>16</sup> with P<sup>238</sup> to Reduce Neutron Yield, Trans. Am Nuc. Soc., Vol. 9, No. 1, 1966, p. 102.Rutherford et al., Preparation of O Reduced in Masses 17 and 18, and Effect on Total Neutrons Emitted from PuO<sup>238</sup>, Trans. Am. Nuc. Soc., Vol. 9, No. 2, 1966, p. 599-600.

McVey, Possible Requirements for Radioisotopes as Power Sources, Nuc. Sci. Abs., Vol. 15, No. 21, 1961, Abs. No. 27914, p. 3600.

Primary Examiner—Carl D. Quarforth

Assistant Examiner—R. L. Tate

Attorney, Agent, or Firm—L. Lee Humphries; Henry Kolin

## [57] ABSTRACT

A primary alpha-particle-emitting radioactive fuel material and a method for preparing it so that secondary neutron generation by an alpha-neutron reaction is substantially reduced. Those individual isotopes of oxygen, carbon, nitrogen, silicon, and chlorine which have a threshold for the alpha-neutron reaction greater than the maximum energy of the emitted alpha particles are selected for combination with the alpha-particle-emitting radioactive isotope to give the desired oxides, carbides, nitrides, silicides, and oxychlorides.

14 Claims, 1 Drawing Figure



PATENTED FEB 5 1974

3,790,440



INVENTOR.  
VAHE KESHISHIAN

By Harry Kolin  
ATTORNEY

## RADIOISOTOPE FUEL MATERIAL AND METHOD

## CROSS REFERENCES TO RELATED APPLICATIONS

This application is a continuation of application Ser. No. 815,131, filed Apr. 10, 1969, which is a continuation-in-part of application Ser. No. 687,945, filed Oct. 25, 1967, which is a division of application Ser. No. 464,702, filed June 17, 1965, now U. S. Pat. No. 3,515,875.

## BACKGROUND OF THE INVENTION

This invention relates to a radioactive fuel material and to a method for preparing such radioactive fuel material for a radioisotope generator. More particularly it relates to an alpha-particle-emitting fuel material for a radioisotope generator wherein neutron shielding requirements are substantially reduced compared with similar generators.

Radioisotope-powered generators are known. Such units are of particular interest for space missions for supplying the power needed by the instruments of the space vehicle. These generators are also of utility in situations where there is need for a remote, unattended, long-lived small power source that is relatively impervious to conditions and hazards of its environment. Such uses include earth-based ones such as navigational aids in remote areas, communication relay stations, forest warning equipment, ocean cable boosters, and the like. This invention is also of interest for use in pacemaker heart devices and artificial hearts which are of medical interest at present for prolonging the life of individuals with certain cardiac deficiencies.

For space missions, particularly manned ones, shielding requirements against radiation contribute significantly to the overall weight of the space vehicle. Astronauts present in the vehicle would require shielding not only from external radiation but also from the radiation emitted by the isotopic power unit itself.

In general, isotopes which are alpha-particle emitters are preferred for fuel use in manned mission space flights because they are relatively easy to shield against, alpha radiation being the least penetrating of all. Exemplary of such a suitable isotopic fuel is plutonium-238. However, the alpha-particle-emitting isotopes are not ordinarily usable as fuel in elemental form, but are present in the form of their compounds, alloys and mixtures so as to provide an isotopic fuel with suitable properties with respect to melting point, hardness, ease of fabrication and handling, and other related physical and metallurgical characteristics.

While alpha-particle emission per se requires but minimal shielding, secondary radiation resulting from interaction of the primary alpha particle with material in the immediate vicinity of the isotope emitter accounts for a significant increase in shielding requirements. The most important secondary source of radiation requiring shielding arises from the alpha-neutron reaction in which an element is transmuted by absorption of an alpha particle, a neutron leaving the excited nucleus.

## SUMMARY OF THE INVENTION

It is an object of this invention to provide an alpha-particle emitter and a method for preparing it whereby there results minimal secondary neutron generation.

In accordance with this invention a novel fuel material is provided having utility in a radioisotope generator which includes a fuel capsule and may include a radiation shield in cooperative relation therewith wherein

5 the radioisotope fuel material is an alpha-particle-emitting radioactive isotope combined with electronegative components which essentially have a threshold for the alpha-neutron reaction greater than the maximum energy of the emitted alpha particles. Thereby 10 secondary neutron generation resulting from an alpha-neutron reaction is substantially reduced, with a corresponding reduction in neutron-shielding requirements. While the radioisotope fuel provided by this invention would not necessarily require a formal shield against 15 neutrons for use in a pacemaker heart device, the reduction of secondary neutron emission would still be of considerable importance.

Preferred as radioisotope fuel materials for use in the practice of this invention are alpha-emitting radioisotopes 20 of the actinide series combined in molecular form with particular low atomic number electronegative elements, or with selected isotopes of these elements, which have a threshold energy for the alpha-neutron reaction greater than the maximum energy of the alpha 25 particles emitted by the radioisotope. Particularly preferred as fuel material is radioactive plutonium oxide wherein the plutonium consists essentially of the plutonium-238 isotope and the oxygen consists essentially of the oxygen-16 isotope substantially free of, or 30 with only trace amounts of, the oxygen-17 and oxygen-18 isotopes. Ordinarily, plutonium-238 oxide will emit a primary neutron by spontaneous fission and about 15 times as many secondary neutrons by an alpha-neutron reaction with natural oxygen. Thus complete elimination 35 of secondary neutrons will reduce overall neutron emission by a factor of 16.

## BRIEF DESCRIPTION OF THE DRAWING

For a more complete understanding of the invention, 40 reference is made to the sole FIGURE of the drawing showing a perspective view, partly in section, of an embodiment of a radioisotope generator suitable for use in practice of this invention.

## 45 DESCRIPTION OF THE PREFERRED EMBODIMENTS

Referring to the drawing, which is intended as illustrative and not restrictive of the present invention, a simplified view of a radioisotope generator 1 is shown 50 from which its principal components may be seen. An outer shell 2, usually in the form of a thin cylindrical can of metal, protects the internal components from contamination and may serve as a heat radiator where required. A radiation shield 3 is required to provide 55 safety requirements in handling the generator during launch and following impact and also to protect astronauts present in the space vehicle during manned space flights. These shields are of high density and prevent the emission of primary and secondary radiation. Exemplary of such shields are lead, depleted uranium, and cast iron. Low density neutron shields such as lithium hydride are also required. These shields all contribute 60 considerably to the weight of the radioisotope generator. This increase in shielding weight is a major disadvantage for space missions. Where the minimizing of shielding weight is a primary consideration, it is preferred to use radioisotopes which are alpha-radiation 65

emitters, since alpha radiation is the least penetrating of all and requires minimal shielding provided no secondary radiation of a penetrating nature occurs.

An energy converter section 4 is used to transform part of the isotope decay heat into electricity. This may consist of an array of thermoelectric elements or thermionic converters. At the heart of the generator is the energy source, shown as a fuel capsule 5 in which a radioisotopic fuel material 6 is enclosed by a capsule wall 7.

The radioisotope generator may be of any desired shape, cylindrical shapes or spherical shapes being more common. In one type of assembly, the energy converters are placed around a space reserved for the fuel capsule. The shield is then wrapped around the converters. The outer shell, except for an end left open for fuel insertion, is soldered or welded around the shield. The fuel capsule is then usually inserted by remote control for safety reasons, and the last piece of the outer shell is then sealed in place. Almost all of the nuclear particles emitted by the decaying radioisotopic fuel are absorbed inside the fuel capsule. During the absorption process, the fast nuclear particles collide with the atoms in the fuel capsule, causing them to move more violently and thus raise the capsule temperature. The kinetic energy of the particles is thereby converted to heat. Generally about 5 to 10 percent of the total heat flow, shown by directional arrows, is converted into electricity. The remaining heat energy produced by the fuel flows into the outer shell from where it is radiated or conducted to a surrounding environment.

Because of the physical and metallurgical requirements for the fuel material, an alpha-particle-emitting isotope cannot ordinarily be used in the pure elemental form. For example, Pu<sup>238</sup> has a melting point ranging from 120°C. to 640°C., depending upon the particular crystalline structure. Whereas, in the form of PuC its melting point is 1654°C.; PuO<sub>2</sub> melts at 2282°C., PuN 2450°C. Similarly, high melting points are shown for ThO<sub>2</sub> 3050°C., ThC 2655°C., UO<sub>2</sub> 2500°C., UN 2630°C. Thus the isotopic materials will ordinarily and preferably be used in the form of their molecular compounds, alloys, or non-stoichiometric mixtures.

It is an essential feature of this invention that secondary neutron generation resulting from an alpha-neutron reaction is substantially reduced by selecting the electronegative component that is combined with the alpha-particle-emitting radioactive isotope to have a threshold for the alpha-neutron reaction that is greater than the maximum energy of the emitted alpha particles. Generally a threshold above about 5.6 Mev is required, this threshold value varying somewhat depending upon the particular alpha-particle-emitting source.

The selection of the particular alpha-particle-emitting radioactive isotope and its combining component will be determined by many factors. As mentioned, metallurgical and physical properties play a primary role. Also of importance is compatibility of the fuel material with cladding materials, as well as its chemical stability, availability and cost. Where a space mission of brief duration is contemplated, an isotope such as polonium-210 which has a half-life of 138 days may be suitable; whereas for a Mars mission, which would require approximately two years, a longer-lived isotope, such as plutonium-238, which has a half-life of

90 years, would be required. Also the choice of isotope would be governed in part by the relative freedom of the alpha-particle-emitting isotope from other primary radiation emission such as gamma rays and neutrons.

The alpha-particle-emitting radioactive isotopes of the actinide series are generally preferred in the practice of this invention. Exemplary of suitable alpha-particle-emitting isotopes are: Pu<sup>238</sup>, Th<sup>228</sup>, U<sup>232</sup>, Cm<sup>242</sup>, Cm<sup>244</sup>, and Am<sup>241</sup>, and also Po<sup>210</sup>. Pu<sub>238</sub> is advantageous for use as an alpha-particle-emitting radioactive source because of its long half-life and the relatively small amounts of gamma rays and neutrons which are also primarily emitted. Thus shielding requirements are considerably minimized. Examples of electronegative components with which the electropositive alpha-particle-emitting isotopes may be combined, either as molecular compounds, alloys, or non-stoichiometric mixtures, are oxides, carbides, nitrides, silicides, and oxychlorides. Preferred fuel materials for the practice of this invention are the oxides, carbides, nitrides, silicides and oxychlorides of the alpha-particle-emitting radioisotopes of the actinide series, e.g., Pu<sup>238</sup>, Th<sup>228</sup>, U<sup>232</sup>, Cm<sup>242</sup>, Cm<sup>244</sup>, and Am<sup>241</sup>, as well as the oxide, nitride, and oxychloride of Po<sup>210</sup>.

In Table I is shown the threshold energy for the alpha-neutron reaction for the relatively light weight natural isotopes. The relative abundance of these natural isotopes is also shown.

TABLE I  
Threshold Energies for Alpha-Neutron  
Reactions in Natural Isotopes from Li to Ni

|    | Isotope          | % Abundance | Threshold Energy for<br>( $\alpha, n$ ) Reaction (Mev) |
|----|------------------|-------------|--------------------------------------------------------|
| 35 | Li <sup>6</sup>  | 7.4         | 4.85                                                   |
|    | Li <sup>7</sup>  | 92.6        | 5.25                                                   |
|    | Be <sup>9</sup>  | 100         | 0 (Q pos.)                                             |
|    | B <sup>10</sup>  | 18.8        | 0 (Q pos.)                                             |
|    | B <sup>11</sup>  | 81.2        | 0.22                                                   |
|    | C <sup>12</sup>  | 98.9        | 11.25                                                  |
|    | C <sup>13</sup>  | 1.1         | 0 (Q pos.)                                             |
| 40 | N <sup>14</sup>  | 99.62       | 6.1                                                    |
|    | N <sup>15</sup>  | 0.38        | 8.15                                                   |
|    | O <sup>16</sup>  | 99.76       | 15.2                                                   |
|    | O <sup>17</sup>  | 0.04        | 0 (Q pos.)                                             |
|    | O <sup>18</sup>  | 0.20        | 0.86                                                   |
|    | F <sup>19</sup>  | 100.0       | 2.35                                                   |
| 45 | Ne <sup>20</sup> | 90.52       | 6.7                                                    |
|    | Ne <sup>21</sup> | 0.27        | 0 (Q pos.)                                             |
|    | Ne <sup>22</sup> | 9.21        | 8.52                                                   |
|    | Na <sup>23</sup> | 100.0       | 3.47                                                   |
|    | Mg <sup>24</sup> | 78.6        | 8.37                                                   |
|    | Mg <sup>25</sup> | 10.1        | 0 (Q pos.)                                             |
|    | Mg <sup>26</sup> | 11.3        | 0 (Q POS.)                                             |
| 50 | Al <sup>27</sup> | 100.0       | 3.05                                                   |
|    | Si <sup>28</sup> | 92.3        | 8.25                                                   |
|    | Si <sup>29</sup> | 4.7         | 1.72                                                   |
|    | Si <sup>30</sup> | 3.0         | 3.95                                                   |
|    | P <sup>31</sup>  | 100.0       | 6.58                                                   |
|    | S <sup>32</sup>  | 95.1        | 9.77                                                   |
|    | S <sup>33</sup>  | 0.74        | 0.75                                                   |
|    | S <sup>34</sup>  | 4.2         | 5.06                                                   |
| 55 | S <sup>36</sup>  | 0.0136      | 3.40                                                   |
|    | Cl <sup>35</sup> | 75.4        | 6.52                                                   |
|    | Cl <sup>37</sup> | 24.6        | 4.28                                                   |
|    | A <sup>40</sup>  | 99.632      | 4.28                                                   |
|    | K <sup>39</sup>  | 93.1        | 7.77                                                   |
|    | K <sup>41</sup>  | 6.9         | 3.72                                                   |
|    | Ca <sup>40</sup> | 96.97       | No data                                                |
| 60 | Ca <sup>42</sup> | 0.64        | 6.58                                                   |
|    | Ca <sup>43</sup> | 0.145       | 0 (Q pos.)                                             |
|    | Ca <sup>46</sup> | 0.0033      | 0.25                                                   |
|    | Ca <sup>48</sup> | 0.185       | 0.15                                                   |
|    | Sc <sup>45</sup> | 100.0       | 2.45                                                   |
|    | Ti <sup>46</sup> | 7.94        | 4.75                                                   |
|    | Ti <sup>47</sup> | 7.75        | 0.38                                                   |
|    | Ti <sup>48</sup> | 73.45       | 2.92                                                   |
| 65 | Ti <sup>49</sup> | 5.52        | 0 (Q pos.)                                             |
|    | Ti <sup>50</sup> | 5.34        | 1.92                                                   |
|    | V <sup>50</sup>  | 0.23        | 0.20                                                   |
|    | V <sup>51</sup>  | 100.0       | 2.45                                                   |

TABLE I—Continued

|                  |       |       |
|------------------|-------|-------|
| C <sup>50</sup>  | 4.49  | 5.30  |
| Cr <sup>52</sup> | 83.78 | 3.85  |
| Mn <sup>55</sup> | 100.0 | 3.80  |
| Fe <sup>54</sup> | 5.81  | 5.95  |
| Fe <sup>56</sup> | 91.64 | 5.43  |
| Fe <sup>57</sup> | 2.21  | 1.4   |
| Fe <sup>58</sup> | 0.34  | 3.84  |
| Co <sup>59</sup> | 100.0 | 5.42  |
| Ni <sup>59</sup> | 67.7  | 10.36 |
| Ni <sup>60</sup> | 26.2  | 8.1   |
| Ni <sup>61</sup> | 1.2   | 4.17  |
| Ni <sup>62</sup> | 3.7   | 6.8   |
| Ni <sup>64</sup> | 1.2   | 4.9   |

In accordance with the teaching of this invention, the electro-negative component forming the oxides, carbides, nitrides, silicides, and oxychlorides will include a mixture of the individual stable isotopes of oxygen, carbon, nitrogen, silicon, and chlorine, these individual isotopes having different thresholds for the alpha-neutron reaction both less than and greater than the maximum energy of the alpha particles emitted by the radioactive isotope. However, this mixture is treated to contain a concentration in greater than its naturally occurring abundance of those ones of the individual isotopes which have a threshold for the alpha-neutron reaction greater than the maximum energy of the emitted alpha particles, i.e., O<sup>16</sup>, C<sup>12</sup>, N<sup>15</sup>, Si<sup>28</sup>, and Cl<sup>35</sup>. Hence, by reacting the electronegative component containing the concentrated isotope with the electropositive component containing the alpha-particle-emitting radioactive isotope, the formed primary alpha-particle-emitting radioactive fuel material will have substantially reduced secondary neutron generation as a result of an alpha-neutron reaction. If the alpha-emitting isotope is used in the form of its carbide, e.g., uranium carbide, the C<sup>13</sup> isotope would be eliminated by chemical or physical treatment either prior to or subsequent to the formation of the compound so that the carbide would be substantially free of the C<sup>13</sup> isotope and would consist almost exclusively of the C<sup>12</sup> isotope, e.g., U<sup>232</sup>C<sup>12</sup>. Thereby, since the threshold energy of the C<sup>12</sup> isotope is 11.25 Mev (Table I), no alpha-neutron reaction would occur and secondary neutron emission would be substantially reduced or eliminated. Similarly, if plutonium oxide (PuO<sub>2</sub>) were used, the radioactive fuel would consist essentially of Pu<sup>238</sup>O<sub>2</sub><sup>16</sup> since the threshold energy of O<sup>16</sup> required for the alpha-neutron reaction is 15.2 Mev; whereas the threshold energy of the O<sup>17</sup> and O<sup>18</sup> isotopes is considerably less. This radioisotope fuel, Pu<sup>238</sup>O<sub>2</sub><sup>16</sup> is particularly preferred therefore in the practice of this invention because of its elimination of secondary neutron generation as well as its desirable chemical and physical properties.

Generally, the desired electronegative isotope will be enriched in greater than its naturally occurring abundance prior to formation of the desired fuel. Thereby, standard chemical reactions which are well known in the art can then be used to prepare the oxides, carbides, nitrides, silicides, and oxychlorides of the desired alpha-particle-emitting radioisotopes of the actinide metals, and the oxide, nitride and oxychloride of polonium. The enriched electronegative isotopes of oxygen, carbon, nitrogen, silicon and chlorine are either available in the form of directly usable compounds, or can readily be converted to usable compounds by standard chemical reactions.

The stable isotopes of the elements of the electronegative component that are utilized for compound forma-

tion are not only selected from the class of oxygen, carbon, nitrogen, silicon, and chlorine isotopes, but also will have present in greater than its naturally occurring abundance those individual isotopes of these electronegative elements which have a threshold for the alpha-neutron reaction greater than the maximum energy of the emitted alpha particles. Referring to Table I, it is seen that the electronegative component would therefore be concentrated in the following isotopes: O<sup>16</sup>, C<sup>12</sup>, N<sup>15</sup>, Si<sup>28</sup> and Cl<sup>35</sup>.

The following enriched isotopes are available from the Isotopes Development Center of Oak Ridge National Laboratory, operated by Union Carbide Corporation for the U.S. Atomic Energy Commission: carbon-12 in inventory form as elemental carbon in an isotopic abundance of greater than 99.9 percent (naturally occurring abundance 98.892 percent); chlorine-35 in the form of NaCl in an isotopic abundance of greater than 98 percent (naturally occurring abundance 75.529 percent); silicon-28 in the form of SiO<sub>2</sub> in an isotopic abundance of greater than 98 percent (naturally occurring abundance 92.21 percent).

Oxygen-16 is obtainable in the form of O<sup>16</sup>-enriched water or O<sup>16</sup>-enriched oxygen gas. Water enriched in the oxygen-16 isotope is obtainable from Volk Isotopes, Westwood, New Jersey, with a depleted content of 0.007 percent O<sup>17</sup> and 0.007 percent O<sup>18</sup>, with the balance O<sup>16</sup>. Oxygen-16 is conveniently obtained in gaseous form by electrolysis of the O<sup>16</sup>-enriched water. The resulting enriched oxygen-16 content is 99.986 percent compared with the naturally occurring abundance in oxygen of 99.759 percent O<sup>16</sup>.

Nitrogen-15 is available from the Isomet Corporation, Palisades Park, New Jersey, in 99 percent enrichment in the form of NH<sub>3</sub>, compared with its naturally occurring abundance of but 0.38 percent. Nitrogen-15 can be prepared by a variety of methods. The Nitrox process involves exchange of NO with HNO<sub>3</sub>. See L. Gowland and T. F. Johns, "A Laboratory-Scale Plant for the Enrichment of <sup>15</sup>N Using the 'Nitrox' Process," AERE-Z/R-2629 (1961), Atomic Energy Research Establishment, Harwell, England. The principal reaction is



Other methods are ammonia-ammonium ion exchange reactions and distillation of NO.

Various standard chemical reactions may be utilized for preparing the desired oxides, carbides, nitrides, silicides, and oxychlorides. Americium metal forms the same compounds with electronegative elements of Group III to VII as do the other actinides. The pink sesquioxide Am<sub>2</sub>O<sub>3</sub> and the black dioxide AmO<sub>2</sub> are known, as well as a number of non-stoichiometric oxides. The dioxide may be obtained by ignition of americium compounds in oxygen-16 gas.

Polonium oxide can be prepared by reacting the metal with oxygen-16 gas at 250°C. according to the reaction



This method for the preparation of the oxide is reported by M. Haissinsky in "Polonium" MLM-1165 (tr)(1964), Mound Laboratories, Miamisburg, Ohio. Thorium and plutonium oxides can be prepared by the same reaction except at a higher temperature, 700°C.

Thorium and plutonium carbides can be prepared by arc-melting the metals with carbon-12, which is the

form supplied by Oak Ridge. The reactions are  $M + C \rightarrow MC$  where  $M$  is plutonium or thorium.

The carbides of americium and of curium may be similarly prepared since both metals have been prepared in macro (multigram) amounts. See L. B. Asprey et al "The Chemistry of the Actinides" Chem. and Eng. News, pages 75-91 (July 31, 1967). Since americium and curium from some of their other reactions are seen to react like true actinides, a straightforward preparation of the carbides would be to arc-melt the metal with the carbon-12 available from Oak Ridge. The reactions are



and



which take place rapidly above the melting point of the carbide. Another standard procedure is to hydride the metals mix with carbon, press and sinter. The reactions are



and



The preparation of americium nitride has been reported by K. Akimoto in J. Inorg. and Nuclear Chem., Vol. 29, pages 2650-2652 (1967) by the reaction  $AmH_2 + NH_3 \xrightarrow{800^\circ} AmN + 2.5H_2$ . Utilizing this reaction, the hydrides of americium and curium may be reacted with ammonia which is supplied 99% enriched in the nitrogen-15 isotope to form the respective nitrides as follows:



Thorium and plutonium nitride can be prepared by reacting the metals with ammonia which is supplied containing nitrogen-15. The reactions are



and



M. Haissinsky, supra, has also reported the preparation of the polonium nitride  $Po_3N_7$  by decomposition of ammonia hexabromo polonite at 200°C.

The standard preparative techniques listed in "Refractory Hard Metals" by P. Schwarzkopf and R. Kieffer, Macmillan, New York, 1953, may be used for the preparation of the actinide metal silicides, i.e., those of Pu, Th, U, Cm and Am. For example, using  $SiO_2$ , the form in which the enriched silicon-28 isotope is available from Oak Ridge, the reaction  $MO_2 + SiO_2 + 4C \rightarrow MSi + 4CO \uparrow$  which is carried out at elevated temperature in vacuum can be utilized. Also, the  $SiO_2$  can be converted to the metal by the reactions



and



The product silicon-28 can then be arc-melted with the metal actinide

- 5  $M + Si \rightarrow MSi$   
as described in the General Procedure and Monthly Progress Report, ANL 6658 (1962), Argonne National Laboratories, Argonne, Illinois.
- 10 The preparation of americium oxychloride is described by G. T. Seaborg and J. J. Katz in The Actinide Elements, New York, McGraw-Hill, 1954, page 513, utilizing the vapor phase hydrolysis of  $AmCl_3$ .

- 15  $AmCl_{3(g)} + H_2O_{(g)} = AmOCl_{(g)} + 2HCl_{(g)}$   
Alternatively, to prepare  $AmOCl$  and  $CmOCl$ ,  $HCl$  gas is prepared from  $NaCl$ , which is supplied by Oak Ridge with enriched  $Cl^{35}$ , by the reaction



- 20 Then the reaction  $AM^{+++}$  (in solution) +  $3(OH)^-$   $\rightarrow Am(OH)_3$  would be carried out followed by  $Am(OH)_3 + 3HCl \rightarrow AmCl_3 + 3H_2O$  using the enriched  $HCl$  gas. The hydrolysis reaction would then be carried

- 25 out using water prepared from oxygen-16,



- according to the procedure outlined above. The same reaction would be used to prepare  $CmOCl$ .

- 30 Plutonium oxychloride can be prepared by the following sequence of reactions:



- 35 using  $HCl$  enriched in chlorine-35.



- 40 using  $H_2O$  enriched in oxygen-16. In the case of thorium, the reactions are



- 45 The  $ThCl_4$  is then heated with water vapor



to give the product.

- 50 All of the thorium and plutonium compounds are discussed in The Actinide Elements, supra.

- 55 Polonium oxychloride  $PoOCl_2$  has been referred to in Nuclear Science Abstracts, Vol. 19, pages 24524 (1965).

- 60 In general, the oxides, carbides and silicides of the actinides are high melting, or stable to high temperature.  $ThO_2$  melts at  $\sim 3000^\circ C$ .,  $PuO_2$  is stable to  $1000^\circ C$ . but apparently converts to a lower oxide above  $1000^\circ C$ .  $Am_2O_3$  and  $Cm_2O_3$  are probably stable to at least  $2000^\circ C$ .  $ThC$  melts at  $2650^\circ C$ .  $PuC$  decomposes above  $1650^\circ C$ . and  $AmC$  and  $CmC$  should be stable to at least this temperature.  $PuSi$  is stable at  $1500^\circ C$ . so the other silicides should also be stable to this temperature. The actinide nitrides probably will decompose above  $1000^\circ C$ . The oxychlorides are in general prepared by hydrolysis with water vapor above  $600^\circ C$ . so they are stable to at least  $500^\circ C$ .

- 65 Maximum benefits in reducing shielding requirements are obtained where there is present as combining

component only the table isotope of the electronegative element which has threshold for the alpha-neutron reaction greater than the maximum energy of the alpha particles emitted by the radioactive isotope. However, substantial improvement in shielding requirements is obtained even where lesser or trace amounts are present of the undesired isotopes which have low threshold values for the alpha-neutron reaction.

For purposes of illustration, without in any sense being limited thereby, a specific method of practicing this invention, and the advantages obtaining thereby, will be illustrated with reference to the radioactive isotopic compounds  $\text{Pu}^{238}\text{O}_2^{16}$  and  $\text{Po}^{210}\text{O}_2^{16}$ .

#### EXAMPLE 1

##### Preparation of Enriched Oxygen-16

Enriched oxygen-16 is conveniently prepared by electrolysis of heavy water,  $\text{D}_2\text{O}$ , which is enriched in the heavier oxygen isotopes. This heavy water process is followed by hydrogen sulfide exchange and then followed by distillation to yield a product containing 90%  $\text{D}_2\text{O}$ . The 90%  $\text{D}_2\text{O}$  is then electrolyzed to produce 99.75%  $\text{D}_2\text{O}$ . During electrolysis, the lighter  $\text{O}^{16}$  isotope comes off initially as a gas, the heavier oxygen isotopes concentrating during this production of  $\text{D}_2\text{O}$  by electrolysis. Using such a process  $\text{H}_2\text{O}$  is obtainable with a depleted content of 0.007%  $\text{O}^{17}$  and 0.007%  $\text{O}^{18}$ , with the balance  $\text{O}^{16}$ . Oxygen-16 is then conveniently obtained in gaseous form by electrolysis of this  $\text{O}^{16}$ -enriched water.

#### EXAMPLE 2

##### Preparation of $\text{Pu}^{238}\text{O}_2^{16}$

###### a. By reaction with Plutonium Metal

Plutonium metal is produced on a continuous basis by electrolysis. The plutonium metal is then heated in  $\text{O}^{16}$  gas at a temperature of 400°C. to form  $\text{PuO}_2^{16}$ .

###### b. From Plutonium Oxide by Hydrofluorination

$\text{PuO}_2$  containing natural oxygen and prepared by low firing at a temperature below 480°C. is converted to  $\text{PuF}_4$  by hydrofluorination at 450°C. The  $\text{PuF}_4$  is reduced to Pu metal by reaction with calcium and iodine. The Pu metal is transferred to a closed system and converted to  $\text{PuO}_2^{16}$  as above described.

###### c. From Plutonium Oxide by Treatment with Phosgene

Plutonium oxide containing natural oxygen is heated at 400°C. with phosgene to convert it to plutonium trichloride. The chloride is then reduced with calcium and iodine to form plutonium metal which is then converted to  $\text{PuO}_2^{16}$  by reaction with  $\text{O}^{16}$  gas as above described.

###### d. From Plutonium Trichloride.

The plutonium trichloride is hydrolyzed in the vapor phase with  $\text{O}^{16}$ -enriched water to form  $\text{PuO}_2^{16}$ . The reaction that occurs is as follows:



#### EXAMPLE 3

##### Decreased Neutron Yield from Alpha-Neutron Reaction

Two samples of radioactive polonium-210 are compared. The samples are obtained as  $\text{PoCl}_4$  deposited on glass. One sample is dissolved in distilled water containing oxygen of natural abundance (99.759%  $\text{O}^{16}$ , 0.037%  $\text{O}^{17}$ , 0.204%  $\text{O}^{18}$ ) and the other in water enriched in  $\text{O}^{16}$  (.007%  $\text{O}^{17}$ , 0.007%  $\text{O}^{18}$ , balance  $\text{O}^{16}$ ). A

small amount of  $\text{HCl}$  is added to both solutions to prevent deposition of  $\text{Po}$  on the walls of the container. The two solutions are then made to the same volume in the same size containers so that the ratio of the count rates observed with a neutron in a fixed geometry is the desired ratio of the neutron production rates. The neutrons from the source solution are thermalized with paraffin so as to permit use of a boron trifluoride neutron detector. This detector is efficient to about 10 percent for neutrons entering the sensitive volume. The cross-sectional area for the detector is selected to be about 20  $\text{cm}^2$ . For a desired count rate of 1,000 counts/min. from the solution of normal water, and a 3-cm thickness of paraffin, about  $10^5$  neutrons/min. is required of the radioisotope source. One curie of  $\text{Po}^{210}$  will produce  $1.33 \times 10^5$  n/min. Using a curie of  $\text{Po}^{210}$  for each of the samples, approximately 1,000 counts/min. is obtained for the solution of normal water and approximately 1,000/30 or about 30 counts/min. for the  $\text{O}^{16}$ -enriched water (i.e.,  $\text{O}^{18}$  depleted water by a factor of 30). Polonium-210 emits alpha particles with an energy of 5.3 Mev, compared with 5.5 Mev for  $\text{Pu}^{238}$ .

According to the data of SERDIUKOVA et al., "Investigation of the  $(\alpha, n)$  Reaction on Oxygen," Bull. Acad. Sci. USSR (Phys. ser.) Vol. 21, p. 1018 (1957), the neutron source from an alpha-neutron reaction on oxygen is proportional principally to the  $\text{O}^{18}$  concentration. In the present process, by depleting both the  $\text{O}^{17}$  and  $\text{O}^{18}$  isotopes, a significant improvement in reducing the emission of secondary neutrons is obtained by using an  $\text{O}^{16}$ -enriched radioactive alpha-emitting oxide.

Where pure  $\text{Pu}^{238}\text{O}_2^{16}$  is used, with the  $\text{O}^{17}$  and  $\text{O}^{18}$  isotopes of oxygen completely eliminated, the overall neutron source can be reduced by a factor of 16. But even with available  $\text{O}^{16}$ -enriched water, where the water is depleted to a content of 0.007%  $\text{O}^{17}$  and 0.007%  $\text{O}^{18}$ , there is a reduction of total neutron emission by a factor of about 10, or a reduction in the secondary alpha-neutron source by a factor of about 27. Thus in one design where an 11-inch thick lithium hydride neutron shield for a  $\text{Pu}^{238}$  oxide isotope source is required using natural oxygen, a reduction in shield thickness to 5 inches is obtained by using the above available  $\text{O}^{16}$ -enriched source. Thus for a space vehicle using as isotope source  $\text{Pu}^{238}\text{O}_2$  containing normal oxygen, the 11-inch thick lithium hydride shield would weigh about 1000 pounds. With  $\text{Pu}^{238}\text{O}_2$  containing the enriched  $\text{O}^{16}$ , 5-inch thick shield weighs about 400 pounds, resulting in a saving in weight of 600 pounds. This reduction in weight is of course highly significant in a space mission.

While the principles of the invention have been described above in connection with specific materials and processes, it is to be clearly understood that this description is made only by way of example and not as a limitation to the scope of the invention as set forth in the objects thereof and in the accompanying claims.

I claim:

1. A primary alpha-particle-emitting radioactive fuel material having a substantially reduced secondary neutron emission by an alpha-neutron reaction comprising a primary alpha-particle-emitting radioactive isotope combined with a component which includes a mixture of individual isotopes of a selected element containing a concentration therein in greater than its naturally occurring abundance of those ones of said individual iso-

topes which have a threshold for the alpha-neutron reaction greater than the maximum energy of the alpha particles emitted by said radioactive isotope whereby secondary neutron generation by said radioactive fuel by an alpha-neutron reaction is substantially reduced.

2. A fuel material according to claim 1 selected from the class consisting of the oxides, carbides, nitrides, silicides, and oxychlorides of plutonium-238, thorium-228, uranium-232, curium-242, curium-244, and americium-241, and the oxide, nitride, and oxychloride of polonium-210, the electronegative component of the radioactive fuel material including a mixture of individual isotopes of an element selected from the class consisting of oxygen, carbon, nitrogen, silicon, and chlorine which contains a concentration therein in greater than its naturally occurring abundance of those ones of said individual isotopes having a threshold for the alpha-neutron reaction greater than the maximum energy of the emitted alpha particles.

3. A fuel material according to claim 2 selected from the class consisting of the oxides of plutonium-238, thorium-228, uranium-232, curium-242, curium-244, americium-241, and polonium-210 wherein the O<sup>16</sup> isotope of the oxygen component is present in a concentration therein in greater than its naturally occurring abundance.

4. A radioactive fuel material according to claim 3 consisting essentially of Pu<sup>238</sup>O<sub>2</sub> wherein the oxygen component is substantially enriched in the O<sup>16</sup> isotope.

5. A radioactive fuel material according to claim 3 consisting essentially of Po<sup>210</sup>O<sub>2</sub> wherein the oxygen component is substantially enriched in the O<sup>16</sup> isotope.

6. A fuel capsule heat source wherein the kinetic energy of nuclear particles emitted by a decaying radio-isotope fuel contained therein is converted to thermal energy, the radioactive fuel material being as set forth in claim 1.

7. A fuel capsule heat source wherein the kinetic energy of nuclear particles emitted by a decaying radio-isotope fuel contained therein is converted to thermal energy, the radioactive fuel material being as set forth in claim 2.

8. A fuel capsule heat source wherein the kinetic energy of nuclear particles emitted by a decaying radio-isotope fuel contained therein is converted to thermal energy, the radioactive fuel material being as set forth in claim 3.

9. A fuel capsule heat source wherein the kinetic energy of nuclear particles emitted by a decaying radio-isotope fuel contained therein is converted to thermal energy, the radioactive fuel material being as set forth in claim 4.

10. A fuel capsule heat source wherein the kinetic energy of nuclear particles emitted by a decaying radio-isotope fuel contained therein is converted to thermal energy, the radioactive fuel material being as set forth in claim 5.

11. The method of preparing a primary alpha-parti-

cle-emitting radioactive fuel material selected from the class consisting of the oxides, carbides, nitrides, silicides, and oxychlorides of plutonium, thorium, uranium, curium and americium, and the oxides, nitride, and oxychloride of polonium for an isotope fuel generator wherein secondary neutron generation by an alpha-neutron reaction is substantially reduced, comprising

providing a first electronegative component for chemical combination with a second electropositive component consisting essentially of a primary alpha-particle-emitting radioactive isotope to form said radioactive fuel material of desired physical and metallurgical properties,

said first component including a mixture of individual isotopes of an element selected from the class consisting of oxygen, carbon, nitrogen, silicon, and chlorine which have different thresholds for the alpha-neutron reaction both less than and greater than the maximum energy of the alpha particles emitted by the radioactive isotope,

said mixture containing a concentration therein in greater than its naturally occurring abundance of those ones of said individual isotopes having a threshold for the alpha-neutron reaction greater than the maximum energy of the emitted alpha particles,

chemically reacting the concentrated first component with said second component consisting essentially of a primary alpha-particle-emitting radioactive isotope selected from the class consisting of Pu<sup>238</sup>, Po<sup>210</sup>, Th<sup>228</sup>, U<sup>232</sup>, Cm<sup>242</sup>, Cm<sup>244</sup>, and Am<sup>241</sup> to form said primary alpha-particle-emitting radioactive fuel material selected from the class consisting of the oxides, nitrides, silicides, and oxychlorides of Pu<sup>238</sup>, Th<sup>228</sup>, U<sup>232</sup>, Cm<sup>242</sup>, Cm<sup>244</sup>, and Am<sup>241</sup> and the oxide, nitride, and oxychloride of Po<sup>210</sup>, and

recovering said radioactive fuel material having a substantially reduced secondary neutron emission by an alpha-neutron reaction.

12. The method according to claim 11 wherein an oxygen component having a natural distribution or the oxygen isotopes oxygen-16, oxygen-17 and oxygen-18 therein is depleted in its oxygen-17 and oxygen-18 content to form an oxygen component substantially enriched in the oxygen-16 isotope, and the enriched component is reacted with a plutonium-238 radioactive isotope to form a radioactive plutonium oxide fuel material wherein said oxide is substantially enriched in the oxygen-16 isotope.

13. The method according to claim 12 wherein said radioactive plutonium oxide fuel material consists essentially of Pu<sup>238</sup>O<sub>2</sub><sup>16</sup>.

14. The method according to claim 12 wherein Pu<sup>238</sup>Cl<sub>3</sub> is hydrolyzed in the vapor phase with O<sup>16</sup> enriched water to form a plutonium oxide fuel material consisting essentially of Pu<sup>238</sup>O<sub>2</sub><sup>16</sup>.

\* \* \* \* \*

UNITED STATES PATENT OFFICE  
CERTIFICATE OF CORRECTION

Patent No. 3,790,440 Dated February 5, 1974

Inventor(s) Vahe Keshishian

It is certified that error appears in the above-identified patent and that said Letters Patent are hereby corrected as shown below:

Column 3, line 22 "capable" should read --capsule-- .

Column 8, the formula on line 34 should read:



Column 9, line 1 "table" should read --stable--; line 2 "haa" should read --has a--.

Column 10, line 61 "radiactive" should read --radioactive--.

Signed and sealed this 16th day of July 1974.

(SEAL)

Attest:

McCOY M. GIBSON, JR.  
Attesting Officer

C. MARSHALL DANN  
Commissioner of Patents